



US005807475A

# United States Patent [19]

Kulprathipanja et al.

[11] Patent Number: 5,807,475

[45] Date of Patent: Sep. 15, 1998

[54] **PROCESS FOR REMOVING SULFUR COMPOUNDS FROM HYDROCARBON STREAMS**

[75] Inventors: **Santi Kulprathipanja**, Inverness; **Laszlo T. Nemeth**, Palatine; **Jennifer S. Holmgren**, Bloomingdale, all of Ill.

[73] Assignee: **UOP LLC**, Des Plaines, Ill.

[21] Appl. No.: **751,829**

[22] Filed: **Nov. 18, 1996**

[51] Int. Cl.<sup>6</sup> ..... **C10G 17/00**

[52] U.S. Cl. ..... **208/208 R**; 208/310 Z;  
208/299

[58] Field of Search ..... 208/208 R, 310 Z,  
208/299

## [56] References Cited

### U.S. PATENT DOCUMENTS

4,634,515 1/1987 Bailey et al. ..... 208/91

4,830,733 5/1989 Nagji et al. ..... 208/208 R  
4,830,734 5/1989 Nagji et al. ..... 208/208 R  
5,114,689 5/1992 Nagji et al. ..... 423/230  
5,114,898 5/1992 Pinnavaia et al. ..... 502/406  
5,117,298 5/1992 Yon et al. ..... 585/823  
5,234,877 8/1993 Pinnavaia et al. ..... 502/84  
5,245,107 9/1993 Yon et al. ..... 585/824  
5,259,946 11/1993 Robinson et al. ..... 208/65  
5,322,615 6/1994 Holtermann et al. ..... 208/91  
5,360,536 11/1994 Nemeth et al. ..... 208/248  
5,520,898 5/1996 Pinnavaia et al. ..... 423/244.04

Primary Examiner—Helane Myers

Attorney, Agent, or Firm—Thomas K. McBride; Frank S. Molinaro

## [57] ABSTRACT

A process for removing sulfur containing compounds from various hydrocarbon streams is disclosed and claimed. The process involves contacting the feedstream with an adsorbent such as nickel exchanged zeolite X or Y, or a smectite layered clay having a surface area of at least 150 m<sup>2</sup>/g, thereby adsorbing the sulfur compounds onto the adsorbent.

**17 Claims, No Drawings**

**PROCESS FOR REMOVING SULFUR COMPOUNDS FROM HYDROCARBON STREAMS**

**FIELD OF THE INVENTION**

This invention relates to a process for removing sulfur containing compounds from various hydrocarbon feedstreams. The process involves contacting the feedstream with an adsorbent such as nickel exchanged zeolite X or a smectite clay, having a surface area of at least 150 m<sup>2</sup>/g, thereby adsorbing the sulfur compounds onto the adsorbent.

**BACKGROUND OF THE INVENTION**

Sulfur and sulfur containing compounds, e.g., H<sub>2</sub>S, mercaptans, organic sulfides and disulfides, etc. are present in crude oil and remain to various degrees in the products obtained from the refining of these crude oils. For example, kerosine and gasoline can contain appreciable amounts of mercaptans which give these products an objectionable odor. One common way to make these products less malodorous is to convert the mercaptans to disulfides. This is known as sweetening. Although sweetening eliminates the mercaptans, it does not remove the sulfur compounds. As stricter pollution control regulations are passed, it is becoming necessary to actually remove the sulfur compounds and not just convert them to less malodorous compounds.

The art discloses a number of processes for removing sulfur compounds from hydrocarbon streams. Many of these processes are aimed at protecting reforming catalysts. For example, U.S. Pat. No. 5,322,615 discloses using an adsorbent which is nickel dispersed on an inorganic oxide support. The support is identified as an amorphous silica bound with alumina.

U.S. Pat. No. 4,634,515 discloses an adsorbent for sulfur compounds which is nickel dispersed on alumina, wherein the nickel crystallite size is at least about 75 Å. U.S. Pat. No. 5,259,946 discloses a process, one step of which involves contacting the hydrocarbon stream with a "sulfur sorbent". The sorbent is a metal dispersed on a refractory inorganic oxide. The metals include zinc, molybdenum, cobalt, tungsten, potassium, sodium, calcium and barium. Inorganic oxide supports include alumina, silica, boria, magnesia and magnesium silicate clays such as attapulgite. U.S. Pat. No. 5,114,898 discloses the use of layered double hydroxide sorbents for removing sulfur oxides from gas streams. Finally, U.S. Pat. No. 5,360,536 discloses a process for removing sulfur containing compounds from liquid organic feedstreams by contacting the feedstream with an adsorbent which is a metal oxide solid solution.

In contrast to this art, applicants have found a series of adsorbents which are particularly effective in removing sulfur containing compounds from a hydrocarbon stream. These adsorbents are nickel zeolite Y, nickel or molybdenum exchanged zeolite X, or a smectite clay having a surface area of at least 150 m<sup>2</sup>/g. Examples of these smectite clays are pillared or delaminated saponites, hectorites and montmorillonites. There is no indication in the art that nickel exchanged zeolite X can be a good sulfur adsorption composition. Further, there is no indication that smectite clays such as saponite or hectorite by themselves are good sulfur adsorbents.

**SUMMARY OF THE INVENTION**

As stated, the present invention relates to a process for removing sulfur compounds from a liquid hydrocarbon

stream. The process comprises contacting the stream at a temperature of about 10° C. to about 100° C. for a time sufficient to adsorb said sulfur containing compounds onto said adsorbent, the adsorbent selected from the group consisting of NiX zeolite, MoX zeolite, NiY zeolite, a smectite layered clay having a surface area of at least 150 m<sup>2</sup>/g and mixtures thereof.

Other objects and embodiments of this invention will become apparent after the following detailed description.

**DETAILED DESCRIPTION OF THE INVENTION**

A variety of hydrocarbon streams can be treated by the process of the instant invention. Generally these streams are those that contain C<sub>6</sub> to C<sub>18</sub> hydrocarbons and include gasoline, kerosine, benzene, toluene, xylene, etc. The sulfur containing compounds which are generally found in these streams and which can be adsorbed onto the adsorbents of this invention include: thiophene, benzothiophene, 2-methylthiophene, 3-methylthiophene, 2-ethylthiophene, n-propyl sulfide, methylethylthiophene, dimethylbenzothiophene, ethyl mercaptan, methyl mercaptan, propyl mercaptan, etc.

The sulfur compounds described above are removed from the hydrocarbon streams by contacting the stream with an adsorbent selected from the group consisting of nickel zeolite Y, nickel exchanged zeolite X, molybdenum exchanged zeolite X, a smectite clay having a surface area of at least 150 m<sup>2</sup>/g and mixtures thereof. Zeolite X belongs to the faujasite family of zeolites. Its synthesis was first reported in U.S. Pat. No. 2,882,244 which is incorporated by reference. Zeolite X has the empirical formula



where M is an alkali or alkaline earth metal, "n" is the valence of M and "Y" has a value up to 8. Briefly, zeolite X is prepared by forming a reaction mixture containing reactive sources of the components, reacting the mixture at a temperature of about 21° C. to about 120° C. for a time of about 1% hours to about 100 hours. Zeolite X is usually synthesized in the sodium form. That is, sodium is the counter ion present in the pores of the zeolite.

The synthesis of zeolite Y is described in U.S. Pat. No. 3,130,007 which is incorporated by reference. Zeolite Y has an empirical formula expressed in terms of moles of oxides of:



where "w" has a value of greater than 3 up to about 6 and "x" has a value up to 9. As with zeolite X, a reaction mixture containing the appropriate ratio of materials is prepared, and then reacted at a temperature of about 20° C. to about 125° C. for a time of about 16 hours to about 8 days.

The nickel or molybdenum forms of zeolites X and Y can be prepared by ion exchange methods well known in the art. Ion exchange can be carried out in a batch or continuous process with a continuous process preferred. In a batch process, the zeolite is mixed with an aqueous solution containing a metal salt (about 1 molar) and the resulting mixture is refluxed for about 2 hours. The mixture is next filtered to isolate the exchanged zeolite. The ion exchange procedure can be repeated until at least 70% exchange and preferably at least 80% exchange is achieved. Additionally, the pH of the solution is adjusted to be between about 4 to about 6. If a continuous process is used, the zeolite is placed

in a column and the metal salt solution is flowed through the column. Again sufficient solution is flowed through the column to effect 70% and preferably 80% exchange of the nickel or molybdenum for the sodium. Regardless of what type of process is used, the metal salts which can be used to carry out the exchange include nickel chloride, nickel nitrate, and sodium molybdate.

Yet another set of adsorbents is the group of clays which make up the smectite family of clays and which have a surface area of at least 150 m<sup>2</sup>/g. Clays are composed of infinite layers (lamellae) of metal oxides and hydroxides stacked one on top of the other. These layers or sheets are composed of tetrahedrally coordinated cations which are linked through shared oxygens to sheets of cations octahedrally coordinated to oxygens and hydroxyls. When one octahedral sheet is linked to one tetrahedral sheet a 1:1 layered structure is formed as in kaolinite, whereas when one octahedral sheet is linked to two tetrahedral sheets, a 2:1 layered structure is produced as in beidellite. Anionic charges on the tetrahedral layers (usually siliceous layers) are neutralized by cations such as Na<sup>+</sup> or Ca<sup>2+</sup> in the interlamellar spaces. These cations can be exchanged with other cations.

The smectite clays are 2:1 layered swellable clays. By swellable is meant that the clays swell or expand when placed in water or other solvents. Specific smectite clays are montmorillonite, beidellite, nontronite, hectorite, saponite and sauconite. The specific formulas for the various smectite clays are presented in Table 1.

TABLE 1

## Formulas of Smectite Clays

| Clay Name       | Formula                                                                                                                |
|-----------------|------------------------------------------------------------------------------------------------------------------------|
| montmorillonite | A <sup>n+</sup> <sub>x/n</sub> Si <sub>8</sub> (Al <sub>4-x</sub> Mg <sub>x</sub> )O <sub>20</sub> (OH) <sub>4</sub>   |
| beidellite      | A <sup>n+</sup> <sub>x/n</sub> (Si <sub>8-x</sub> Al <sub>x</sub> )(Al <sub>4</sub> )O <sub>20</sub> (OH) <sub>4</sub> |
| nontronite      | A <sup>n+</sup> <sub>x/n</sub> (Si <sub>8-x</sub> Fe <sub>x</sub> )(Fe <sub>4</sub> )O <sub>20</sub> (OH) <sub>4</sub> |
| hectorite       | A <sup>n+</sup> <sub>x/n</sub> (Si <sub>8</sub> )(Mg <sub>6-x</sub> Li <sub>x</sub> )O <sub>20</sub> (OH) <sub>4</sub> |
| saponite        | A <sup>n+</sup> <sub>x/n</sub> (Si <sub>8-x</sub> Al <sub>x</sub> )(Mg <sub>6</sub> )O <sub>20</sub> (OH) <sub>4</sub> |
| sauconite       | A <sup>n+</sup> <sub>x/n</sub> (Si <sub>8-x</sub> Al <sub>x</sub> )(Zn <sub>6</sub> )O <sub>20</sub> (OH) <sub>4</sub> |

The value of x varies from about 0.2 to about 1.8. A is a counter ion selected from the group consisting of alkali metals, alkaline earth metals, secondary amines, tertiary amines, quaternary ammonium cations and quaternary phosphonium cations and n is the charge on said counter ion.

These clays either occur naturally or can be synthesized. Usually the smectite clays are hydrothermally synthesized from a reaction mixture containing the required molar amounts of the desired metals. The reaction mixture contains reactive sources of the desired metals such as sodium aluminate, aluminum hydroxide, boehmite alumina, gibbsite alumina, aluminum isopropoxide, aluminum t-butoxide, colloidal silica, tetraethylorthosilicate (TEOS), tetramethylorthosilicate, magnesium sulfate, magnesium fluoride, lithium fluoride, iron chloride, zinc sulfate and zinc chloride. The counter ion is added as a salt or compound. Examples of the metal salts are sodium hydroxide, lithium hydroxide, potassium hydroxide, cesium hydroxide and calcium hydroxide. Examples of quaternary compounds are the hydroxide, chloride, iodide, bromide and carbonate salts of the following cations: tetramethylammonium; tetraethylammonium; tetrapropylammonium; tetrabutylammonium; tetra-t-butylammonium; tetrapentylammonium; tetraphenylammonium; tetramethylphosphonium; tetraethylphosphonium; tetrapropylphosphonium and tetraphenylphosphonium. Illustrative of the secondary and tertiary amines which

can be used are di-n-propylamine, ethylbutylamine, tripropylamine, triethylamine, piperidine, 2-methylpyridine, di-n-pentylamine, choline and N,N-dimethylbenzylamine. The pH of the reaction mixture can range from about 5 to about 14 and the mixture reacted at a temperature of about 50° C. to about 250° C. under autogenous pressure for a time of about 2 hours to about 21 days to crystallize the desired clay.

Usually the clays either as synthesized or as they occur in nature do not have sufficient surface area to be used as adsorbents in the present process. As stated, the clay must have a surface area of at least 150 m<sup>2</sup>/g. The surface area of the clays can be increased by either delaminating the clay or pillaring the clay. Both methods are well known in the art. Delamination is accomplished by exchanging the clay with various inorganic salts such as NH<sub>4</sub>Cl, AlCl<sub>3</sub>, CrCl<sub>3</sub>, FeCl<sub>3</sub>, NH<sub>4</sub>OH, etc. and then drying quickly by means such as flash drying, spray drying or freeze drying. Pillaring of the clay means propping the clay layers open with large cations (oligomers) of Fe<sup>3+</sup>, Cr<sup>3+</sup>, or metal hydroxy polymer cations such as (Al<sub>13</sub>O<sub>4</sub>(OH)<sub>24</sub>(H<sub>2</sub>O)<sub>12</sub>)<sup>7+</sup> or (Zr(OH)<sub>2</sub>•4H<sub>2</sub>O)<sup>8+</sup>. Upon drying and calcining as described below, Fe<sub>2</sub>O<sub>3</sub>, Cr<sub>2</sub>O<sub>3</sub>, Al<sub>2</sub>O<sub>3</sub> or ZrO<sub>2</sub> pillars are obtained. Other examples of pillars include TiO<sub>2</sub>, SiO<sub>2</sub> and Si/Al (amorphous silica-alumina). These pillars are introduced by combining the clay with an oligomer or polymer of the desired cation or mixture of cations at reaction conditions. For example, alumina pillars may be introduced by using aluminum chlorohydrate (ACH). Aluminum chlorohydrate (also known as aluminum chlorohydroxide) is a polymeric metal complex having the empirical formula



where n has a value of about 4 to 12. The preparation of this aluminum polymer is generally known to those skilled in the art. See, for example: Tsuitida and Kobayashi, *J. Chem. Soc. Japan* (Pure Chem. Sect.), 64, 1268 (1943). Inoue, Osugi and Kanaji, *J. Chem. Soc. Japan* (Ind. Chem. Sec.), 61, 407 (1958).

A rare earth ACH is an ACH as described above which is modified to include one or more rare earth elements such as cerium, lanthanum, neodymium, europium, etc. The ACH polymer is modified with the rare earth by adding a soluble rare earth salt, preferably a water soluble rare earth salt. Examples of rare earth salts are the nitrates, halides, sulfates and acetates. Preferred rare earth elements are cerium and lanthanum with cerium nitrate and lanthanum nitrate being the preferred salts. The rare earth is introduced into the polymer or oligomer structure by mixing the rare earth salt either in solution (water preferred) or as a solid with the ACH. The resulting solution is refluxed at a temperature of about 105° C. to about 145° C. for a time of about 24 to about 100 hours. The weight ratio of rare earth (expressed as oxide, e.g., CeO<sub>2</sub>) to alumina (Al<sub>2</sub>O<sub>3</sub>) in the solution prior to refluxing is from about 1:52 to about 1:1.

Descriptions of the other pillaring materials can be found in the following references: 1) Si/Al—U.S. Pat. No. 4,176,090; 2) zirconia—*Clays and Clay Minerals*, 27, 119 (1979) and U.S. Pat. No. 4,176,090; 3) titania—U.S. Pat. No. 4,176,090; 4) chromium oxide—U.S. Pat. No. 4,216,188 and 5) silicon oxide—U.S. Pat. No. 4,367,163, all of which are incorporated by reference.

These pillared clays are prepared by means well known in the art such as adding the smectite clay to a solution containing the pillar or a pillar precursor, stirring, filtering, redispersing with water (one or more times), isolating, drying and calcining at about 300° C. to about 800° C. for a time sufficient to fix the structure (preferably about 16 hours).

Contacting of the liquid hydrocarbon stream with any of the adsorbents described above can be carried out by means well known in the art. For example, the contacting can be carried out in a batch mode or in a continuous mode. In a batch mode, the stream to be treated is mixed with a sufficient amount of adsorbent in an appropriate size reaction vessel. The resultant mixture can be stirred or agitated to ensure complete contact of the stream with the adsorbent. In order to ensure that the sulfur compounds are completely adsorbed onto the support, it is necessary that the hydrocarbon stream be contacted with the solid solution for a time of about 10 minutes to about 10 hours. If a continuous process is used, the adsorbent is placed in a vertical column and the stream to be treated is upflowed through the column. The stream is flowed at a liquid hourly space velocity of about 0.1 to about 10 hr<sup>-1</sup>.

Whether the process is carried out in a batch or continuous manner, the adsorbent can be used in the form of extrudates, pills, beads, spheres, etc. Usually, the adsorbent is mixed with a binder such as attapulgite clay, minugel clay and bentonite clay and then formed into the desired shape. The amount of binder which is used varies from about 8 to about 20 wt. %. Processes for forming the various shapes are well known in the art.

Finally, the contacting can be carried out over a broad temperature range. Generally the temperature range is from about 10° C. to about 100° C. with a range of about 20° C. to about 70° C. being preferred. The process is conducted at atmospheric pressure or pressures up to 1379 kpag (ga) (200 psig).

The following examples are presented in illustration of this invention and are not intended as undue limitations on the generally broad scope of the invention as set out in the appended claims.

#### EXAMPLE 1

An aqueous nickel solution was prepared by adding 110 gm of  $\text{NiCl}_2 \cdot 6\text{H}_2\text{O}$  to 500 mL of deionized water. This solution was flowed through 100 mL of a NaY zeolite adsorbent column at 75° C. The effluent solution was recycled through the column for 16 hours to convert the NaY zeolite to NiY zeolite. At this point the column was washed with 500 mL of deionized water, the adsorbent was unloaded from the column, dried at 50° C. for 5 hours and then calcined at 350° C. for 3 hours. This sample was designated sample A.

#### EXAMPLE 2

ANiX zeolite was prepared as per Example 1, except that NaX was used instead of NaY. This sample was designated sample B.

#### EXAMPLE 3

AMoX zeolite was prepared as per Example 2 except that the ion exchange solution was prepared by mixing 110 gm of  $\text{Na}_2\text{MoO}_4 \cdot 2\text{H}_2\text{O}$  into 500 ml of deionized water. This sample was designated sample C.

#### EXAMPLE 4

A saponite clay was prepared as follows. In a 2,000 mL 3-neck round bottom flask equipped with a condenser, an overhead stirrer and a thermometer there were placed 378 g of  $\text{MgSO}_4 \cdot 7\text{H}_2\text{O}$  and 510 g of deionized water. After heating the flask to 85° C., there was added a solution of 377.6 g of

water glass (29.95%  $\text{SiO}_2$ ), and 10.3 g of NaOH in 259 g of deionized water with heavy mixing. The resulting slurry was stirred for 60 minutes at which time there was added a solution of 62 g  $\text{Na}_2\text{CO}_3 \cdot \text{H}_2\text{O}$ , 82 g NaOH, 29.6 g  $\text{NaAlO}_2$  and 500 g of deionized water. After stirring for an additional 60 minutes the slurry was transferred to a liner, placed in a Parr reactor and crystallized at 200° C. for 8 hours. The product was recovered by filtration and washed with 2 liters of water and then dried at 110° C. X-ray diffraction analysis of the product showed it to be a poorly crystallized smectite clay. The BET surface area of the clay was 320 m<sup>2</sup>/g.

The saponite clay described above was now ammonium exchanged as follows. In a 2,000 ml beaker, 55 g of  $\text{NH}_4\text{Cl}$  were dissolved in 1,000 ml of water. To this solution there were added 25 g of the delaminated saponite clay. The resultant mixture was stirred for 30 minutes and then left quiescently for 24 hours. Next the clay was recovered by filtration and the entire procedure repeated. Finally, the clay was washed with 2 liters of deionized water, dried at 110° C. and then calcined at 300° C. for 2 hours. The BET surface area of the clay was 260 m<sup>2</sup>/g. This sample was identified as sample D.

#### EXAMPLE 5

A pillared hectorite clay was prepared as follows. First a cerium aluminum chlorohydrate (ACH) pillar was prepared by mixing 4.8 g  $\text{Ce}(\text{NO}_3)_3 \cdot 6\text{H}_2\text{O}$  with 66 g of ACH sol (obtained from Reheiss Corporation) in a teflon liner. The liner was placed in a Parr reactor and the reactor was placed in a 135° C. oven and held there for 5 days.

In a 3,000 ml 3-neck round bottle flask equipped with a condenser, an overhead stirrer and a thermometer, there were placed 2,100 g of deionized water and 137 g of Ce-ACH sol prepared above. The flask was heated to 95° C. and after 30 minutes 54 g of hectorite clay (obtained from American Colloid and identified as Hectolite GM®) was added while stirring. The resultant slurry was heated at 95° C. for 1 hour with stirring at which point the solid was recovered using a centrifuge. The clay was next washed with water until chloride free and dried at 60° C. for 16 hours and then calcined at 600° C. for 2 hours. X-ray diffraction analysis showed that the clay had been pillared and nitrogen absorption analysis showed that the clay had a BET surface area of 550 m<sup>2</sup>/g. This sample was identified as sample E.

#### EXAMPLE 6

A Ce-ACH pillared montmorillonite clay was prepared as in Example 5 except that montmorillonite identified as HPM-20® was obtained from American Colloid. This sample was identified as sample F.

#### EXAMPLE 7

The adsorbents in Examples 1-6 were tested for their sulfur adsorption properties using the following test procedure. In a container there were placed 0.5 g of the adsorbent and 3 g of gasoline and the mixture maintained at ambient temperatures for 16 hours. The starting gasoline was found to contain 345 ppm of sulfur. After 16 hours the adsorbent was separated from the gasoline and the gasoline tested for sulfur. The results of this test are presented in Table 2.

TABLE 2

| Sulfur Adsorption of Various Adsorbents |                           |                          |                  |
|-----------------------------------------|---------------------------|--------------------------|------------------|
| Sample I.D.                             | Adsorbent                 | Sulfur Content*<br>(ppm) | % Sulfur Removal |
| A                                       | NiY                       | 207                      | 40.0             |
| B                                       | NiX                       | 173                      | 49.8             |
| C                                       | MoX                       | 178                      | 48.4             |
| D                                       | NH <sub>4</sub> -Saponite | 161                      | 53.3             |
| E                                       | Ce-ACH Hectorite          | 194                      | 43.7             |
| F                                       | Ce-ACH Montmorillonite    | 192                      | 44.3             |

\*Sulfur content of gasoline after contact with adsorbent for 16 hours.

We claim as our invention:

1. A process for removing sulfur containing compounds from a liquid hydrocarbon stream comprising contacting the stream at a temperature of about 10° C. to about 100° C. for a time sufficient to adsorb said sulfur containing compounds onto said adsorbent, the adsorbent selected from the group consisting of NIX zeolite, MoX zeolite, NiY zeolite, a smectite layered clay having a surface area of at least 150 m<sup>2</sup>/g, and mixtures thereof.
2. The process of claim 1 where the process is carried out in a continuous mode.
3. The process of claim 2 where the stream is contacted with the adsorbent at a liquid hourly space velocity of about 0.1 to about 10 hr<sup>-1</sup>.
4. The process of claim 1 where the process is carried out in a batch mode.
5. The process of claim 4 where the stream is contacted with the adsorbent for a time of about 10 minutes to about 10 hours.

6. The process of claim 1 where the adsorbent is NiX zeolite.
7. The process of claim 1 where the adsorbent is MoX zeolite.
- 5 8. The process of claim 1 where the adsorbent is NiY zeolite.
9. The process of claim 1 where the smectite layered clay is a delaminated smectite layered clay selected from the group consisting of delaminated saponite, delaminated 10 hectorite, delaminated montmorillonite, delaminated beldellite, delaminated nontronite and delaminated saucomite.
10. The process of claim 9 where the smectite clay is delaminated saponite.
- 15 11. The process of claim 9 where the smectite clay is delaminated hectorite.
12. The process of claim 9 where the smectite clay is delaminated montmorillonite.
13. The process of claim 1 where the smectite layered clay 20 is a pillared smectite clay, said pillar selected from the group consisting of Al<sub>2</sub>O<sub>3</sub>, rare earth containing Al<sub>2</sub>O<sub>3</sub>, ZrO<sub>2</sub>, TiO<sub>2</sub>, Cr<sub>2</sub>O<sub>3</sub>, SiO<sub>2</sub> and silica/alumina.
14. The process of claim 13 where the pillar is rare earth containing Al<sub>2</sub>O<sub>3</sub>.
- 25 15. The process of claim 1 where the adsorbent is in the shape of pellets, extrudates or beads.
16. The process of claim 15 where the shaped adsorbent contains from about 8 to about 20% of a binder.
17. The process of claim 16 where the binder is selected 30 from the group consisting of attapulgite clay, minugel clay and bentonite clay.

\* \* \* \* \*

UNITED STATES PATENT AND TRADEMARK OFFICE  
**CERTIFICATE OF CORRECTION**

PATENT NO. : 5,807,475  
DATED : Sep. 15, 1998  
INVENTOR(S) : KULPRATHIPANJA et al.

It is certified that error appears in the above-identified patent and that said Letters Patent is hereby corrected as shown below:

In Claim 1, line 21, "of NIX zeolite" should be corrected to read --of NiX zeolite--.

Signed and Sealed this

Twenty-ninth Day of December, 1998

Attest:



BRUCE LEHMAN

Attesting Officer

Commissioner of Patents and Trademarks